

## UNITED STATES PATENT OFFICE

2,079,860

## CARROTING FUR

Hans O. Kauffmann, Buffalo, N. Y., assigner to  
Buffalo Electro-Chemical Company, Inc.No Drawing. Application November 23, 1934,  
Serial No. 754,541

10 Claims. (Cl. 6—21)

This invention relates to a carotting composition and to a process of carotting fur.

In the preparation of felt hats the fur from which the felt is prepared must be preliminarily treated to induce the requisite felting properties of the fur. The procedures whereby the fur, generally rabbit's fur or "coney", is rendered suitable for use in the preparation of felt have been generally designated as carotting.

10 It is generally accepted in the hatting industry that a good felt can be prepared only from fur that has been carotted with mercury nitrate in some form. The mercury carrot as used heretofore is prepared by adding metallic mercury to nitric acid in prescribed proportions, permitting the reaction between the acid and the mercury to proceed to completion diluting with water to the desired Baume and thereafter brushing the resulting solution upon the fur, permitting the treated fur to dry, and thereafter cutting the fur from the skin and felting the fur into hat forms.

It has been proposed from time to time to employ non-mercurial carotting solutions for treating fur preparatory to the felting operation; in substantially every case the use of the non-mercurial solutions has been abandoned after a short trial. It would appear that proper felting qualities are imparted to the fur by the mercury salt and nitric acid as those carotting solutions in which these materials are constituents, have been the only solutions which have enjoyed any long continued commercial use.

Extreme precautions must be observed in the preparation and use of mercury nitrate carrot since the mode of application of the carrot to the fur must be such that the hair or fur is moistened with the solution from the tip to the base, but such moistening, usually done by brushing the solution upon the fur, must be done in such manner so as not to apply too great an excess of the carotting solution to the fur, otherwise the hair or fur may be damaged, burned or discolored, and with white skins should the discoloration be excessive, the fur is not suitable for the preparation of hats in the light colors or pastel shades. In general white skins cannot be carotted practically with the usual mercury-nitric acid carrot.

The present invention provides a carotting 50 composition containing a metal salt and nitric acid that can be applied to fur to produce carotted fur showing substantially no discoloration of the fur; the final carotted fur showing a minimum of reds, yellows and browns upon the tips 55 of the hair. The instant invention also provides

a carotting solution that can be used to produce fur suitable for use in the preparation of hats in the lighter shades of color. Other advantages of the present invention will become apparent in the following description of the composition and process and will be particularly pointed out in the claims appended hereto.

In the preparation of the carotting composition of the present invention mercury and nitric acid are permitted to react in proportions sufficient to produce a mercury carrot of the usual composition, the proportions of nitric acid and mercury being varied over a considerable range, depending upon the type of skin to be treated, and upon the type of cut fur it is desired to produce. To this solution is added a substance capable of removing non-nitric nitrogen compounds, the quantity of the material being sufficient to effect the removal of such non-nitric nitrogen compounds that may be present in the solution or that may be developed during the subsequent drying operation to which the skins are subjected after the application of the carrot and which discolor the fur. A mercury carrot of general application is one of specific gravity of about 13° Bé.; the amount of the non-nitric nitrogen destroying material added is from about 0.1% to about 10%, this quantity generally being sufficient to destroy the nitrogen compounds producing discoloration of the fur.

Metals having the power of combining with nitric acid and which in contact with the acid fur-cleaning and hydrolyzing agent cooperate therewith to produce properly carotted fur, may be substituted for mercury in the new carrot, due allowance being made for differences in their combining weights with respect to mercury. As examples of such metals lead, tin, bismuth and silver may be mentioned as metals whose nitric acid solutions possess the necessary cleaning, 40 hydrolyzing and carotting action upon fur to produce a fur capable of being wetted and felted.

The new carrot of the present invention, therefore, is acid in reaction and contains a metal nitrate with substantially no nitrous acid or lower oxides of nitrogen dissolved in the solution, all the brownish gas being destroyed and the yellowish color, sometimes present in the mercury carrot, being eliminated. The carotting solution, therefore, of the present invention contains an acid hydrolyzing agent for cleaning and modifying some constituent substance of or on the fur fiber whereby the fur fiber can be wet when immersed in hot water, this wetting characteristic not being present to any substantial extent in un- 55

carroted fur. The new carrot of the present invention also contains an added material capable of removing substances present in the usual mercury nitrate carrot imparting deleterious color to the fur, such added material being present in quantity sufficient to remove such discoloring agents originally present in the solution, and also those subsequently formed during the hydrolyzing or cleaning action as well as those produced during the drying operation. I have found that color preventing agents are generally reducing agents in the sense that these substances reduce or render inactive the non-nitric nitrogen compounds or other color imparting compounds that may be present in the solution or subsequently formed during the course of the carrottting; including the application of carrot to the skin and during the drying of the skin with the applied carrottting solution upon it.

In carrying out the process of the present invention I preferably apply the carrottting solution to the skin by brushing the same into the fur prior to cutting the fur from the skin. The treated skins are stacked and dried and the fur thereafter removed from the skin and made into felt. Skins once carrottted and dried in accordance with this procedure do not deteriorate but may be kept until it is decided to cut the fur from the skin and to have it used for felt making.

As a reducing agent or non-nitric nitrogen compound removal agent, I have found hydroxylamine, in the form of one of its salts, as for instance the sulfate, particularly efficacious; the resulting carrottting composition contains a carrottting metal nitrate, free nitric acid and the reducing agent to prevent the action of the color imparting materials upon the fur with resultant discoloration thereof.

As a further exemplification of the diversity of combination that may be suitably employed, depending upon the type of fur to be treated, the type of fur to be produced, or depending upon manufacturing conditions, temperature conditions employed in the particular manufacturing operation or upon the humidity pertaining within a particular manufacturing plant, the strength and concentration of the carrottting solution may be varied over a considerable range.

As illustrative of the range of composition the following are given by way of example:

- (1) To 100 parts of a 7° Baumé solution of mercury nitrate is added  $\frac{1}{6}$  part of hydroxylamine sulphate.
- (2) To 100 parts of a 13° Baumé mercury nitrate solution is added 4 parts of hydroxylamine sulphate.
- (3) To 100 parts of 20° Baumé solution of mercury nitrate is added 12 parts of hydroxylamine sulphate.

As stated above, the preferred range of combination and the one suitable for employment with the type of skin generally encountered will be a 7 to 18° Baumé mercury nitrate containing from about 0.1 to about 10% of the reducing agent, the quantity of reducing agent in any case being an amount sufficient to eliminate the material imparting color to the fur during the carrottting and subsequent drying. Substances other than hydroxylamine can be employed, and I have found that urea, thio urea, carbamide and the like may be suitably employed in this connection. Other substances that can be suitably added to prevent the formation of reds and yellows upon the fur are hydrazine as well as certain of its derivatives and also materials or substances re-

acting with the lower oxides of nitrogen, such as ammonia salts, for instance, ammonium chloride. Guanidine also possesses the property of eliminating the color imparting substances. The preparation of the carrottting solution of the present inventor is preferably effected with hydroxylamine or other reducing agent not producing the white precipitate within the solution that is formed when hydrazine, urea and some of their derivatives are added as reducing agents to the mercury nitrate solution.

Examples merely illustrative of the use of other carrottting meals and reducing agents are:

(1) To 100 parts of an 8° Baumé lead nitrate solution is added 2½ parts of hydroxylamine sulfate.

(2) To 100 parts of a 12° Baumé silver nitrate solution is added 4 parts of guanidine sulfate.

(3) To 100 parts of a 15° Baumé bismuth nitrate solution is added 5 parts of urea.

From a consideration of the above, it will be apparent that the present invention provides a carrottting solution containing a carrottting metal nitrate and a hydrolyzing and cleansing agent acidic in nature, capable of changing the fur fibers from a non-wetting fiber to a fiber capable of being wet with water; the fiber retains its initial and original strength, has not been partially oxidized and destroyed but is readily felted and produces a good shrinking fur. The white fur carrottted in accordance with the process of the present invention is not discolored with reds and yellows to such an extent that it may not be used for the production of the lighter shades of felts.

It will further be seen that the invention provides a carrottting composition wherein the fur coloring agents have been removed from the solution prior to the application of the carrottting composition to the fur, and a composition possessing the ability to eliminate any color imparting substances formed during the action of the carrottting composition upon the fur or during the subsequent drying of the fur. In addition, fur carrottted with the composition of the present invention is not burned or rendered harsh and brittle upon the tips but remains soft and possesses a good feel and possesses good shrinking qualities necessary for proper felting.

What is claimed is:

1. A carrottting solution comprising an aqueous solution of mercury nitrate, hydroxylamine and nitric acid.
2. A carrottting solution comprising the reaction product of a reducing agent containing an amino group and a solution of mercury nitrate acid in reaction, of at least 3° Baumé strength.
3. The process of carrottting fur which comprises subjecting the fur to the action of an aqueous carrottting solution of mercury nitrate, hydroxylamine and nitric acid.
4. The process of carrottting fur which comprises subjecting the fur to the action of an aqueous carrottting solution of mercuric nitrate acid in reaction mixed with a reducing agent containing an amino group.
5. A carrottting solution comprising an aqueous solution of a carrottting metal salt hydroxylamine and nitric acid.
6. A carrottting solution comprising an aqueous solution of a carrottting metal salt, a reducing agent containing an amino group and nitric acid.
7. A carrottting solution comprising the reaction product of a reducing agent containing an amino group and a solution of a carrottting metal

nitrate, acid in reaction, of a strength of 18° Baume or less.

5 8. The process of carotting fur which comprises subjecting the fur to the action of an aqueous carotting solution of a carotting metal nitrate, a reducing agent containing an amino group and nitric acid.

9. A carotting solution comprising an aqueous solution of lead nitrate, a reducing agent containing an amino group and nitric acid.

10. A carotting solution comprising an aqueous solution of silver nitrate, a reducing agent containing an amino group and nitric acid. 5

HANS O. KAUFFMANN.